

(Model.)

R. SCHIMMEL.

PROCESS OF MANUFACTURING CHAIR SEATS OF VEGETABLE  
FIBER AND CHROMIC ACID.

No. 297,639.

Patented Apr. 29, 1884.

Fig. 1.



Fig. 2.



Fig. 3.



Fig. 4.



Witnesses.

John F. Allen

J. Gammel, Jr.

Inventor.

Rudolf Schimmel  
per Harry E. Strode  
Attorney.

# UNITED STATES PATENT OFFICE.

RUDOLF SCHIMMEL, OF ANNABERG, GERMANY.

## PROCESS OF MANUFACTURING CHAIR-SEATS OF VEGETABLE FIBER AND CHROMIC ACID.

SPECIFICATION forming part of Letters Patent No. 297,639, dated April 29, 1884.

Application filed May 25, 1883. (Model.)

*To all whom it may concern:*

Be it known that I, RUDOLF SCHIMMEL, a citizen of Germany and a resident of Annaberg, in Germany, have invented a new and 5 Improved Chair-Seat, of which the following is a specification.

Figures 1 and 2 are perspective views of the product; Fig. 3, a cross-section. Fig. 4 represents a side view of compressing device.

10 The nature of my invention consists of a mixture of pulp of ground rags and vegetable fiber, in equal parts, and chromic acid, made in a thick mass or paste, from which sheets of the required shape and design are formed for covering the seats and backs of chairs and similar articles of furniture, as a substitute for cane or wood seats. The vegetable fibers, preferably of wood, and the ground rags are worked and mixed in a pulping-engine, with the addition 20 of chromic acid, three parts to one hundred parts of water, and this thick mass or paste is then formed into sheets of the required size and thickness. The thus-formed sheets may be strengthened by the addition of a textile 25 material of linen, cotton, or any other material placed in the central part of the sheet. The sheet, after being cut in the desired size and shape, is then placed between two plates, C D, of which the lower plate, D, has a straight 30 surface, and the upper plate, C, has the design or pattern engraved or cut on its surface,

which is desired to be given to the sheet, and is likewise provided with projecting pins to perforate the sheet. These plates C D, with the sheet between them, are then passed between pressure-rollers E F, whereby the desired configuration is given to the surface of the sheet, as shown in Figs. 1 and 2, or of any other desired design. The thus molded and pressed sheet is then varnished, to protect the 35 same against moisture and the changes of the temperature, and after being dried will be ready for use. These sheets can be made to represent cane-seats of any desired design, and will be found very strong, durable, and cheap. 40

45 What I claim as my invention, and desire to secure by Letters Patent, is—

The process of manufacturing chair-seats, consisting of the following steps: first, mixing together ground rags and vegetable fiber (in 50 equal parts) and chromic acid to make a paste; then forming this paste into sheets; then strengthening these sheets by the addition of textile fabric; then molding and pressing each sheet to give the proper texture and superficial configuration; then varnishing and drying 55 each sheet and cutting the chair-seats out of the same.

RUDOLF SCHIMMEL.

Witnesses:

GUSTAV SCHÄDTLER,  
PAUL RAUH.